

# UNITED STATES PATENT OFFICE.

CHILD HAROLD WILLS, OF DETROIT, MICHIGAN.

## SPRING-STEEL.

1,288,345.

Specification of Letters Patent. Patented Dec. 17, 1918.

No Drawing. Original application filed June 19, 1917, Serial No. 173,719. Divided and this application filed August 7, 1917. Serial No. 184,942.

*To all whom it may concern:*

Be it known that I, CHILD HAROLD WILLS, a citizen of the United States, residing at Detroit, in the county of Wayne and State 5 of Michigan, have invented certain new and useful Improvements in Spring-Steels, of which the following is a specification.

This invention relates to spring steels for use in the manufacture of springs for automobiles and the like, and it is a division of 10 my copending application, Serial Number 173,719 filed June 19th, 1917.

It is one of the primary objects of my invention to provide a spring steel which will 15 have a maximum resistance to alternating stresses and, at the same time, have superior physical properties. Among the other objects of my invention is the provision of a steel having the characteristics described 20 which is economical to manufacture, easily worked, and which has an increased range of heat treatment temperatures, the advantages of which will hereinafter be more fully set out.

25 In the usual classes of spring steel at present in use, difficulties have been encountered in a number of important respects. In the first place it is impossible in such steels to obtain maximum resistance to alternating 30 stresses, and at the same time obtain maximum physical properties, for the reason that the resistance to alternating stresses increases as the annealing temperature approaches the critical point, while the physical properties decrease. If the carbon content be increased to increase the physical 35 properties, the liability to cracking when the steel is quenched and the development of other defects and undesirable characteristics 40 are increased. Furthermore, the range of temperature within which such steels must be treated is very narrow which of course, frequently results in losses in manufacture 45 and failure in service, because of the difficulty of maintaining furnace temperatures uniform. By my present invention I overcome the foregoing difficulties, obtain a greatly increased range of temperature for 50 heat treatment and the steels at the same time have superior depth hardening characteristics.

I accomplish the foregoing by adding to spring steel, molybdenum in small percentages, preferably from a substantial fraction of 1% up to about 1%. I find that such

molybdenum spring steel can be manufactured more economically than ordinary spring steels for the reason that the molybdenum increases the yield by decreasing the amount of cropage or discard and the 60 amount of grinding necessary. This results from the fact that the tendency to seam or to pipe is greatly reduced, and in addition, the molybdenum does not segregate and apparently overcomes the tendency of the other 65 alloying elements to segregate, which of course, causes the steel to run more uniformly throughout. From the steel makers' standpoint, therefore, such molybdenum is not only economical to make but it is superior in quality.

In so far as manufacture is concerned, the steel is superior for the reason that the molybdenum greatly increases the temperature range for heat treatment and thus 75 obviates the necessity for complicated furnace regulating equipment, and greatly reduces the losses ordinarily incurred when the allowable limits of temperature are exceeded. In ordinary steels when the narrow 80 range of temperature is exceeded, the properties of the steel are greatly impaired, but in steel made in accordance with my invention, the ordinary range of heat treatment can be greatly exceeded without detrimental 85 structural and chemical change. At the same time the steel is readily workable and has superior depth hardening characteristics, as above noted. As a result of the increase in temperature range, the steel runs 90 uniformly.

With regard to the article produced, *i. e.*, the performance of the springs, the use of molybdenum not only increases the resistance to alternating stresses but also greatly 95 increases the physical properties, so that the springs will be strong enough to support the load and withstand shock without permanent setting. To illustrate, in spring steels made in accordance with my invention, a 100 tensile strength varying from 201,000 pounds to 270,000 pounds, elastic limit varying from 180,000 pounds to 225,000 pounds, elongation from 7% to 15%, and reduction of area from 17% to 45% may be 105 obtained. It will be noted that the tensile strength, and the elastic limit, in view of the elongation and reduction of area percentages obtained, are very marked, the superiority of the steel being all the more em- 110

phasized by the fact that the resistance to alternating stresses without crystallization is greatly increased, and by the fact that the molybdenum increases the depth of hardening. Notwithstanding these greatly increased physical properties, the steel is readily workable.

In carrying out my invention I prefer the following analyses as giving the most satisfactory results, namely, carbon from .38% to .55%; manganese from .40% to 1.25%; chromium from a fraction of a per cent. to 2%; silicon from .10% to .40%; and molybdenum in substantial fractional percentages up to 1%. I find that if the molybdenum content be materially carried above 1% the steel develops undesirable characteristics. It will also be understood that the manganese and chromium may be replaced by equivalent elements or omitted, but these are preferred because the molybdenum in-

tensifies the effect of the other alloys, particularly the chromium. I also prefer to draw the steel at temperatures ranging approximately from 1020° F. to 1100° F., or 25 stated in other words, I prefer to draw materially above the temperatures at which full blue and dark blue colors manifest themselves.

I claim:

1. Heavy duty spring steel containing molybdenum in quantities not materially exceeding 1% and drawn materially above 320° C.

2. Spring steel carbon from .38% to .55%; 35 manganese from .40% to 1.25%; chromium from a fraction to 2%; silicon from .10% to .40%; and molybdenum from a fraction to 1%, substantially as set forth.

In testimony whereof I have hereunto signed my name.

CHILD HAROLD WILLS.